

## UNITED STATES PATENT OFFICE.

CARL CRAMER, OF ZURZACH, SWITZERLAND.

## BLEACHING EARTH.

No Drawing.

Application filed February 27, 1922. Serial No. 539,714.

*To all whom it may concern:*

Be it known that I, CARL CRAMER, a citizen of the Swiss Republic, and resident of Zurzach, Switzerland, have invented new and useful Improvements Relating to Bleaching Earths, of which the following is a full, clear, and exact specification.

For bleaching or decoloring animal, vegetable and mineral oils and fats, large quantities of earthy matters having bleaching properties are used. Such mineral matters consist in the main of aluminium hydro-silicates and are found in large quantities in various places. They are known in trade under such names as Forida earth, floridin, fuller's earth. Frequently, however, it is not the natural material which is used, this material being first subjected to a preliminary treatment. Such treatment is for the purpose of enhancing the bleaching power of the mineral; it may consist in cautious heating to expel hygroscopic water, or in treating the mineral with an acid such as hydrochloric or sulfuric acid. Products of this kind are those known as tonsil and frankonit.

In practice, the crude material is treated with hydrochloric acid of about 15% strength. This operation known as opening up, generally lasts for two hours, and is carried out at boiling temperature, that is to say, by continuous injection of steam.

According to the present invention, this opening up can be achieved in a surprisingly short time by emulsifying the material with an acid of 1% strength in the cold. This emulsification or homogenizing may be effected for instance with the aid of known homogenizing apparatus, comprising at least one centrifugal wheel as, for instance, a turbomixer capable of producing an emulsification of an intensity sufficient to enhance notably, already by itself, the bleaching

power of the aluminium hydro-silicates, even when their emulsifying would be performed with water alone, that is to say, without the aid of an acid. The product thus prepared is particularly well opened up both chemically and physically has a more powerful bleaching effect than any of the known products. Apart from this important fact, there is the great advantage in practice that fuel and the greater part of the acid hitherto used are saved.

The following example illustrates the invention:—

1,000 kilos of an earth of the kind in question are stirred with 3,000 litres of hydrochloric acid of 1% strength in a wooden vat provided with a stirrer, and are emulsified with the aid of the known turbo mixer. After ten minutes the charge is drained, washed with water and then dried in a drying oven.

What I claim is:—

1. A process for obtaining bleaching earths having a high bleaching effect by treating aluminium hydro-silicates with an acid, consisting in mixing the aluminium hydro-silicates with dilute hydrochloric acid and emulsifying the resulting mixture intensely in the cold.

2. As new products, bleaching earths having a high bleaching effect, the said bleaching earths having been opened up chemically and physically by their emulsification with dilute hydrochloric acid in the cold, substantially as set forth.

In witness whereof I have hereunto signed my name this 10th day of February, 1922, in the presence of two subscribing witnesses.

CARL CRAMER.

Witnesses:

FRIEDRICH KURZ,  
AMAIN GRANN.